

# UNITED STATES PATENT OFFICE.

ROBERT A. HADFIELD, OF SHEFFIELD, ENGLAND.

## MANUFACTURE OR TREATMENT OF STEEL ARMOR-PLATES.

No. 834,904.

Specification of Letters Patent.

Patented Nov. 6, 1906.

Application filed April 14, 1906. Serial No. 311,788.

*To all whom it may concern:*

Be it known that I, ROBERT A. HADFIELD, a subject of the King of Great Britain, and a resident of Sheffield, county of York, England, have invented an Improvement in the Manufacture or Treatment of Steel Armor-Plates and the Like, of which the following description, in connection with the accompanying drawing, is a specification, like letters on the drawing representing like parts.

This invention has for its object the production of an improved process or mode of treatment for cast-steel armor-plate shields and the like with plain, corrugated, or other faces, and the invention can be applied to the treatment of other articles of steel, whether or not having hard surfaces.

In a pending application, Serial No. 283,235, filed by me October 18, 1905, I have described an improvement in the manufacture of cast-steel armor-plates with corrugated faces. The present application is an improvement for carrying forward the method or process of treatment therein set forth.

In carrying out my present invention I have in practice obtained satisfactory results by the following mode of procedure: A mold is prepared from a pattern of appropriate dimensions and of the proper form, and said mold can be made of fire-resisting sand dried in the usual manner. Upon one of its edges (the article to be produced being preferably cast vertically) the head or feeding portion is located. The metal used may advantageously be steel prepared in a manner similar to that described in the specification of my British Letters Patent No. 16,132, of 1901. After pouring, and preferably while the casting is still hot, it is removed to a furnace, where it is allowed to cool down slowly in order to prevent internal strains, after which the sand is removed and the casting carefully cleaned.

In the case of a shield, plate, or other article, which I shall hereinafter refer to for the sake of brevity as a "plate," requiring to be rendered hard on one or more of its surfaces such plate is suitably carburized where required. For example, the plate is put into a furnace, and upon the surface of the plate is placed a suitable carburizing medium, such as charcoal. The temperature of the furnace is then raised to, say, between 900° centigrade and 1,100° centigrade, and the plate is allowed to remain in the furnace for several days, the actual period in a given case de-

pending upon the extent to which the carburizing is to be carried. The plate is then allowed to gradually cool down in the furnace, and the head or riser is removed in the usual manner by being slotted off. I then heat the plate to from 700° centigrade to 850° centigrade, usually preferring about 760° centigrade, after which the plate is cooled down as far as desired, either slowly in the furnace or it may be air-cooled, and it is then reheated to between 700° centigrade and 850° centigrade and cooled to between 640° centigrade and 690° centigrade, after which the plate is wholly or partially quenched in water, depending upon the size and shape of the article, due care being taken that the plate is not allowed to remain too long in the water to produce a greater degree of hardness or stiffness than required. After this quenching the plate is again heated to between 570° centigrade and 640° centigrade, the preferable temperature depending upon the composition of the steel, and it is allowed to cool in the furnace. It is then reheated to between 570° centigrade and 640° centigrade and quenched outright, preferably in water, after which it may be taper-heated—that is, heated so that the face assumes a temperature of from 700° centigrade to 770° centigrade, tapering to a temperature at the back of the plate of from 400° centigrade to 600° centigrade—whereupon the plate is dipped in or sprayed with oil or water, according to the hardness required. Inasmuch as the face is hotter than the back, the face will become hard, while the back remains soft and tough. In some cases—as, for example, when a very soft steel is being treated, *i. e.*, one low in carbon—a uniform instead of a taper heating may be adopted.

If the plate does not require to be face-hardened, the carefully-cleaned casting is placed in a furnace, which is then raised to a high temperature—say 900° centigrade and 1,100° centigrade—the plate being withdrawn from the furnace as soon as the requisite temperature has been reached. The head or riser is then removed.

The remaining steps in the treatment for a plate that is not face-hardened are the same as for a face-hardened plate, as hereinbefore set forth except that the taper-heating is omitted when producing a plate that is not face-hardened.

The heat treatment hereinbefore described, with or without carburization and with or

without the taper-heating, may be applied to various kinds of steel, whether cast or forged.

The details of the process hereinbefore set forth may be more or less modified in different particulars by those skilled in the art without departing from the spirit and scope of my invention.

Having described my invention, what I claim as new, and desire to secure by Letters Patent, is—

1. In the manufacture of steel armor-plate, shields and the like, gradually raising the temperature of the article to from 900° centigrade to 1,100° centigrade and allowing the article to gradually cool down; then heating said article to from 700° centigrade to 850° centigrade and cooling slowly and reheating to between 700° centigrade and 850° centigrade, and cooling to between 640° centigrade and 690° centigrade, and quenching; reheating after quenching to between 570° centigrade and 640° centigrade and cooling; repeating the heating to not more than 640° centigrade, and then quenching.

2. In the manufacture of steel armor-plate, shields and the like, gradually raising the temperature of the article to from 900° centigrade to 1,100° centigrade and allowing the article to gradually cool down; then heating said article to from 700° centigrade to 850° centigrade and cooling slowly, and reheating to between 700° centigrade and 850° centigrade and cooling to between 640° centigrade and 690° centigrade, and quenching; reheating after quenching to between 570° centigrade and 640° centigrade and cooling; repeating the heating to not more than 640° centigrade and then quenching; then taper-heating the article, raising the temperature of the face thereof higher than the temperature of the back, and dipping or spraying with oil or water.

3. In the manufacture of steel armor-plate, shields and the like, subjecting the plate to a temperature of from 900° centi-

grade to 1,100° centigrade while the face thereof is in contact with carbonaceous material, and maintaining the plate subjected to such temperature for several days; then allowing the plate to gradually cool down; reheating it to from 700° centigrade to 850° centigrade and cooling slowly, and reheating to between 700° centigrade and 850° centigrade and cooling to between 640° centigrade and 690° centigrade, and quenching; reheating after quenching to between 570° centigrade and 640° centigrade and cooling, repeating the heating to not more than 640° centigrade, and then quenching.

4. The herein-described process of making steel armor-plate, shields and the like, which consists in casting the same in a mold, slowly cooling the casting in a furnace, and thereafter removing and cleaning the casting; subjecting the casting for several days to a furnace-temperature of from 900° centigrade to 1,100° centigrade while in contact with carbonaceous material, and then allowing the plate to gradually cool down in the furnace; then heating the casting to from 700° centigrade to 850° centigrade and cooling slowly; repeating the last-named step and then cooling the casting to between 640° centigrade and 690° centigrade, and quenching the casting in water; reheating to between 570° centigrade and 640° centigrade and cooling; repeating the last-named heating, and then quenching the casting; then taper-heating such casting to a temperature of from 700° centigrade to 770° centigrade at its face, tapering to from 400° centigrade to 600° centigrade at the back, and dipping or spraying with oil or water.

In testimony whereof I have signed my name to this specification in the presence of two subscribing witnesses.

ROBERT A. HADFIELD.

Witnesses:

LUTHER J. PARR,  
CHAS. N. DANIELS.